

United States Patent [19]  
Kuniyasu et al.

[11] 3,713,477  
[45] Jan. 30, 1973

[54] METHOD OF MANUFACTURING  
METALLIC SHORT FIBERS

[75] Inventors: Yoshihiro Kuniyasu, Kawasaki,  
Akio Matsumoto, Eiji Isobe, both of  
Tokyo; Kenji Someno, Tokyo, all  
of Japan

[73] Assignee: Mitsui Mining & Smelting Co., Ltd.  
Tokyo, Japan

[22] Filed: Feb. 26, 1971

[21] Appl. No.: 119,196

[30] Foreign Application Priority Data

June 22, 1970 Japan ..... 45/54185

[52] U.S. Cl. ..... 164/69, 164/82, 264/176 F

[51] Int. Cl. ..... B22d 11/12

[58] Field of Search ..... 164/69, 81, 82, 283;  
264/176 F

[56] References Cited  
UNITED STATES PATENTS

|           |        |                 |             |
|-----------|--------|-----------------|-------------|
| 2,825,108 | 3/1958 | Pond.....       | 164/82 UX   |
| 2,879,566 | 3/1959 | Pond.....       | 164/81 X    |
| 2,904,859 | 9/1959 | Wade et al..... | 164/273 R X |
| 2,976,590 | 3/1961 | Pond.....       | 164/82      |

FOREIGN PATENTS OR APPLICATIONS

1,168,521 9/1958 France ..... 164/82

OTHER PUBLICATIONS

Zeitshrift fur Metallkunde, 27(5), 1935. TN3Z5, pp.  
114-115.

Primary Examiner—R. Spencer Annear  
Attorney—Woodhams, Blanchard and Flynn

[57] ABSTRACT

A method of manufacturing metallic short fibers comprising the steps: making the melt flow out through a small orifice under elevated pressure; and making the resulting solidified endless metallic fiber run against a slant cooling device to thereby break it into pieces of fixed length.

5 Claims, 1 Drawing Figure



PATENTED JAN 30 1973

3,713,477



INVENTORS  
YOSHIHIRO KUNIVASU  
AKIO MATSUMOTO  
EIJI ISOBE  
KENJI SOMENO  
BY  
Wardhamer, Blackard & Flynn  
ATTORNEYS

## METHOD OF MANUFACTURING METALLIC SHORT FIBERS

### BACKGROUND OF THE INVENTION

#### a. Field of the Invention

The present invention relates to an improvement in the method of manufacturing metallic short fibers by flowing molten metal through a small orifice under elevated pressure and then solidifying same.

#### b. Description of the Prior Art

The conventional methods of manufacturing various metallic fibers through mechanical processes such as the extrusion process, wire-drawing process, etc. are exclusively intended for obtaining an endless fiber, while, as to the manufacturing of metallic short fibers of uniform length, no pertinent method has ever been developed. As a result, in case where metallic short fibers are required, such as for preparing a composite material by means of mixing metallic short fibers, for the purpose of reinforcement, with another substance or producing porous pressure-moldings by the use of metallic short fibers, it has been usual to employ the method in which conventional endless fibers are cut into pieces of a fixed length to serve for said purpose by means of a cutter. However, this method of cutting endless fibers has been defective in that it is poor in productivity due to the complicated process and apparatus, that the quality of the metallic short fibers thus obtained is such that the surface of the fiber gets stained or distorted caused by working or a multiplicity of short fibers are caused to adhere to each other by the cut ends under pressure even after cutting, thereby forming a bunch inconvenient for handling, etc.

On the other hand, in case of the melt spinning process which comprises the steps that a melt obtained by fusing a metal is made to flow out through a small orifice at the bottom of a receptacle by applying mechanical force, pneumatic pressure or the like and the melt thus flowing out is solidified by means of an appropriate cooling atmosphere, thereby producing a metallic fiber, though it is admittedly possessed of improved productivity as compared with the mechanical process such as the extrusion process, wire-drawing process, etc. mentioned above and the metallic fiber obtained thereby is also superior in quality, the product resulting from this conventional method has also been confined to endless fibers.

### SUMMARY OF THE INVENTION

The present inventors have conducted a series of researches on the properties and behaviors of the melt for use in the foregoing melt spinning process and confirmed the fact that a metallic fiber immediately after solidification of the melt flowed out from a small orifice is so poor in intercrystal bonding strength that application of just a slight force readily brings about separation of crystals and breakdown of the fiber. This phenomenon is called the state of hot shortness. They also noticed the fact that a metallic fiber descending in such a state as above can be made into metallic short fibers of uniform length by means of applying thereto a regular breaking force, and, based on this observation, they have successfully achieved their object by means of making the metallic fiber collide with a slant metallic plate as a means of giving rise to regular breaking force and taking advantage of the bending stress arising from said collision.

In other words, the present invention relates to a method of manufacturing metallic fibers by means of making a melt flow out through a small orifice under elevated pressure, which comprises the step that an endless metallic fiber being made of the melt thus flowing out and in the state of hot shortness immediately after solidification thereof is made to collide with a slant cooling device to be broken into pieces of uniform length.

10

### DESCRIPTION OF THE PREFERRED EMBODIMENTS

Referring to the appended drawing which is a schematic representation of apparatus to be utilized in practicing one embodiment of the present invention, 1 denotes the receptacle, 2 denotes the small orifice provided in the bottom of said receptacle, 3 denotes the cooling device and 4 denotes the collecting box. The melt A in the receptacle 1 is subjected to elevated pressure applied thereon by an appropriate means, so that it flows out through the small orifice 2 at a regular speed and gets solidified completely at the point marked B. On this occasion, if there no cooling device 3 is provided, the melt thus flowing out will be collected in the form of an endless fiber. According to the present invention, however, by virtue of the provision of the slant cooling device 3, the descent of the solidified metallic fiber C is obstructed as the tip D thereof collides with the cooling device 3, and, as a result, the metallic fiber C bends as shown in the drawing, is subjected to a bending stress, and finally gives way under this bending stress to break at the point marked E. The metallic short fibers F resulting from such breaking slip down 15 along the cooling device 3 to be collected in the collecting box 4. The length of the metallic short fibers F to be obtained in this way can be controlled at will by means of modifying the distance between the point marked E and the point marked D: the closer the point 20

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

5290

5295

5300

5305

5310

5315

5320

5325

5330

5335

5340

5345

5350

5355

5360

5365

5370

5375

5380

5385

5390

5395

5400

5405

5410

5415

5420

5425

5430

5435

5440

5445

5450

5455

5460

5465

5470

5475

5480

5485

5490

5495

5500

5505

5510

5515

5520

5525

5530

5535

5540

5545

5550

5555

5560

5565

5570

5575

5580

5585

5590

5595

quite suitable material for use in manufacturing porous board-type mold goods. Moreover, since the present short fibers are absolutely free from any permanent set inasmuch as they have been subjected to cooling subsequent to the breaking in the state of hot shortness and are possessed of a uniform texture, the function of the manufactures made by utilizing them is improved.

As the material for the melt in the present invention, lead, zinc, aluminum, lead base alloys, zinc base alloys and aluminum base alloys are all applicable.

The metallic short fibers made by the present invention can be made into porous molded goods through pressure-molding process by taking advantage of the above-mentioned properties to serve as the electrode plate of battery, catalyst, filter, sound-arresting material, etc. and they also can be mixed with synthetic resins as a material for use in preparing a composite having the electric conductivity and thermal conductivity.

#### EXAMPLE 1

Pure lead was melted at 360°C, and the melt thus prepared was made to flow out under a pressure of 2.0 kg/cm<sup>2</sup> through a nozzle having a sectional area of 0.01 mm<sup>2</sup> at the speed of 5.5 m/sec onto a stainless-steel plate for the purpose of breaking and cooling the descending lead fiber, which plate was disposed 15 cm below the bottom of the nozzle with a gradient of 60°. By means of thus making the lead fiber collide with said stainless-steel plate, there were obtained short fibers of pure lead with a length of 2 mm, which were separated from each other without being intertwined and possessed of a quite clean surface.

#### EXAMPLE 2

Lead-4 percent antimony alloy was melted at 320°C, and the melt thus prepared was made to flow out under a pressure of 2.0 kg/cm<sup>2</sup> through a nozzle having a sectional area of 0.008 mm<sup>2</sup> onto a stainless-steel plate which was disposed 15 cm below the bottom of the nozzle with a gradient of 60°, whereby the descending lead fiber was broken into pieces and there were obtained short fibers of lead-4 percent antimony alloy with a length of 1.5 mm each at the rate of about 20,000 pieces per minute. Further, by means of disposing said stainless-steel plate at a position 20 cm below the bottom of the nozzle, there were obtained short fibers of said alloy with a length of 7 mm each.

#### EXAMPLE 3

Pure zinc was melted at 450°C, and the melt thus prepared was made to flow out under a pressure of 1.0 kg/cm<sup>2</sup> through a nozzle having a sectional area of 0.04 mm<sup>2</sup> and to collide with a hollow copperwork of water-cooling type which was disposed 2.0 m below the bottom of the nozzle with a gradient of 45°, whereby there were obtained short fibers of pure zinc with a length of 2 mm each.

#### EXAMPLE 4

An aluminum alloy containing 11 percent silicon was melted at 620°C, and the melt thus prepared was made to flow out under a pressure of 2.0 kg/cm<sup>2</sup> through a nozzle having a sectional area of 0.09 mm<sup>2</sup> and to collide with a hollow copperwork of water-cooling type which was disposed 2.5 m below the bottom of the nozzle with a gradient of 30°, whereby there were obtained short fibers of said alloy with a length of 3 mm each.

All the short fibers prepared as above displayed fluidity like a metallic powder and could be readily filled in a metal pattern uniformly. A porous board manufactured by the process of pressure-molding upon filling the present fibers in a 2 cm square metal pattern was possessed of an apparent density of 4.0 and displayed uniform density all over the structure including all the edges and corners thereof.

What is claimed is:

1. A method of manufacturing short metal fibers, which comprises:

continuously extruding molten metal substantially vertically downwardly through a small orifice under elevated pressure to form a continuous, downwardly moving filament;

immediately after the filament leaves the orifice, cooling the filament to solidify same without breaking same so that the solidified portion of the filament remains integral with the molten metal issuing from the nozzle, so that there is formed in the solidified portion of the filament a zone of increased brittleness at a position spaced downwardly from said orifice;

continuing to move the filament substantially vertically downwardly and directing the lowermost tip of the solidified portion of the filament against the smooth upper surface of a target member, which surface is inclined with respect to the vertical, to bend the solidified filament and thereby to cause the filament to break substantially at said zone of increased brittleness to form a short fiber;

and continuing to move said filament so that the lowermost tip thereof is repeatedly directed against said surface whereby said filament is repeatedly broken into short fibers.

2. A method according to claim 1, in which said member is made of metal and is maintained stationary during the method.

3. A method of manufacturing metallic short fibers according to claim 1, wherein said member is vertically and horizontally adjustable.

4. A method of manufacturing metallic short fibers according to claim 1, wherein said member is a hollow metalwork of water-cooled type.

5. A method of manufacturing metallic short fibers according to claim 1, wherein the metal is selected from the group consisting of lead, zinc, aluminum, lead base alloys, zinc base alloys and aluminum base alloys.

\* \* \* \* \*